

## UNITED STATES PATENT OFFICE.

JOHN MERLE HOSDOWICH, OF JERSEY CITY, NEW JERSEY, ASSIGNOR TO CHROMIUM PRODUCTS CORPORATION, OF WILMINGTON, DELAWARE, A CORPORATION OF DELAWARE.

## PROCESS OF PLATING WITH CHROMIUM.

No Drawing.

Application filed September 10, 1925. Serial No. 55,622.

This invention relates to process of chrome plating; and it comprises a method of producing hard, dense and continuous coatings of chromium by electro-deposition 5 wherein a chrome plating bath containing chromate of chromium receives an addition of a salt of a metal more negative than chromium in the electrochemical series, such as iron, and bath conditions are so adjusted 10 as to deposit chromium practically to the exclusion of the other metal; all as more fully hereinafter set forth and as claimed.

The properties of the metal render it valuable as a surface coating for other softer 15 and more corrodible metals; and various processes, and notably that of Grube, Patent No. 1,496,845, are in use for producing such a coating by plating from an aqueous bath. In the Grube bath, chromic acid ( $\text{CrO}_3$ ) is 20 present and is used for replenishment as the bath loses chromium. From these baths, chromium coatings may be electrically deposited having all the desirable properties. The best of the baths contain chromium in 25 two states of oxidation, as  $\text{CrO}_3$  and as hydrated  $\text{Cr}_2\text{O}_3$  and the two oxids may be combined as chromate of chromium.

While these processes are good and produce good coatings they require skill in use 30 and are open to improvement in "throwing power;" which for the present purposes is the property producing even coatings irrespective of surface configuration in the cathode. With any electroplating bath there 35 is always a tendency for a deposit to occur preferentially on projecting portions of an article forming a cathode as compared with hollows, crevices and sheltered portions. The better the throwing power of a bath, 40 the more this tendency is restrained.

In the course of an extensive series of experiments on improving the throwing power of these baths by various addition agents, organic and inorganic, the unexpected discovery was made that throwing power as 45 regards chromium was considerably improved by the presence in the bath of various other metals more negative than chromium in the electrochemical series; that is, by the presence of metals which normally are more readily plated out of solution than is chromium itself. In a bath containing  $\text{CrO}_3$  and chromate of chromium however

and of the right pH concentration, these other metals do not deposit and on the other hand chromium is thrown down in coatings of desirable properties both from a physical and chemical point of view. Deposits may be had ranging in color from bright highly lustrous metal through a frosted condition and down to a dull gray. Unexpectedly the voltage required is lower than that heretofore considered necessary in the deposition of chromium from these chromic acid baths and the cathode current efficiency is higher. The deposits obtained are substantially pure chromium in spite of the presence of the other metal which is normally more easily reducible.

It has been found that the phenomenon in question exists with all the salts of the heavy metals more negative than chromium in the electrochemical series when present in certain definite concentrations. The salts may be added to the bath as sulfates, chlorides, bromides, carbonates, etc., and the amount present may vary from less than a gram per liter up to about 30 grams per liter, that is, about 3 per cent.

In the present invention I employ for the deposition of chromium an electrolyte containing chromium chromate and salts of another metal in proportions within the stated range. The pH concentration of the bath should be such as to insure an excess of chromium hydroxid over the amount necessary to neutralize any free acid other than  $\text{CrO}_3$  present in the electrolyte, while the concentration of  $\text{CrO}_3$  should be at least twice that of the hydrated  $\text{Cr}_2\text{O}_3$  and of the metallic salt used. Under these conditions, the bath contains chromium chromate and there is a sufficient concentration of chromium ions to permit free deposition of chromium. Insoluble anodes such as lead or oxids thereof may be used or there may be used soluble anodes of chromium, chromium alloys or chromium and another metal in mechanical admixture.

In a typical embodiment of the present invention an electrolytic solution is prepared containing  $\text{CrO}_3$  and chromium hydroxid together with a small proportion of ferrous sulfate. A good bath may be prepared by dissolving 325 grams of  $\text{CrO}_3$  in the necessary volume of water, heating to

boiling and then stirring into the hot solution 12 grams of commercial hydrated chromic oxid,  $\text{Cr}(\text{OH})_3$ . When the latter is completely in solution 6 grams of commercial 5 hydrated ferrous sulfate,



is added and allowed to dissolve. The whole mixture is now diluted to the volume of a 10 liter and is ready for electrolysis. A bath made up in this way with the proportions stated is introduced into a suitable electrolytic cell which is advantageously fitted with a coil for heating and cooling. The best 15 temperature for electrolysis of this solution is between 35 and 45° C. A suitable voltage is from 2.5 to 5 volts; the particular voltage depending on the size of the cathode, its shape and the thickness of deposit desired. 20 Ordinarily it is desirable to have a current density of 0.05 to 0.2 amperes per square centimeter. During electrolysis solid  $\text{CrO}_3$  is added from time to time so as to keep the 25 chromium content of the electrolyte substantially unchanged. Since the iron is not thrown down no replenishment of this is necessary except as regards mechanical losses.

In practice the bath is analyzed from time 30 to time and if the amount of iron present is found decreased to any material extent

more ferrous sulfate is added. Instead of using ferrous sulfate as in the above example other metallic salts may be employed. With nickel sulfate similar results are obtained. Chromium plating from a bath containing nickel sulfate to the extent of 6 grams per liter (0.6%) with 325 grams of  $\text{CrO}_3$  and 12 grams of  $\text{Cr}(\text{OH})_3$  on analysis shows no trace of nickel. Like results 40 are obtained where the bath receives an addition of sulfates, chlorides, etc., of cadmium, tin, lead, antimony, bismuth, copper and mercury.

What I claim is:—

1. In the production of chromium plating baths of better throwing power, the process which comprises adding a small proportion of a soluble salt of a metal more negative than chromium in the electrochemical series 50 to a chromium plating bath containing chromium in two stages of oxidation.
2. A process such as described in claim 1, where the salt added is a salt of iron.
3. A process such as described in claim 55 1, wherein the amount of metal salt present together with the amount of chromium in the lower state of oxidation is not more than one-half the concentration of  $\text{CrO}_3$ .

In testimony whereof I affix my signature.

JOHN MERLE HOSDOWICH.